

June 7, 1927.

1,631,528

W. F. HENDRY

DRY CELL

Filed Jan. 23, 1924.

*Fig. 1.*



*Fig. 2.*



INVENTOR  
W. F. Hendry  
BY *Panekoski*  
his ATTORNEY

## UNITED STATES PATENT OFFICE.

WILLIAM F. HENDRY, OF OSSINING, NEW YORK, ASSIGNOR, BY MESNE ASSIGNMENTS, TO NATIONAL CARBON COMPANY, INC., OF NEW YORK, N. Y., A CORPORATION OF NEW YORK.

## DRY CELL.

Application filed January 23, 1924. Serial No. 688,058.

This invention relates to dry cells and more particularly to a novel method of providing a separating lining between depolarizing mixtures and anode surfaces.

5 The present invention is in the nature of an improvement on my copending United States Patent No. 1,597,232, dated August 24, 1926, in which a multiple cell is provided with the anodes connected in multiple 10 and a common cathode, the depolarizing mixtures of the various cells being in the form of compacted tablets. In order to separate the anode from the depolarizing tablets a paper wrapper is provided around 15 each tablet, preferably a coating of paste being applied to the paper.

In order to avoid the necessity of providing these separate paper wrappers, in accordance with the present invention a coating of bibulous material, serving to separate the depolarizing mixture from the anode, 20 is provided in the form of a coating adhering to the tablets themselves. This is preferably accomplished by compacting the tablets of alternate layers of wood pulp, or other bibulous material, and depolarizing mixture, the relative quantities being such 25 as to form a coating of bibulous material around the core of depolarizer. Presses are well known in the art, e. g., tablet making 30 machines for pharmaceutical preparations in which a coating of sugar is compacted around a core of other material and simultaneously with the compacting thereof.

35 In the present case, the coating is accomplished by first delivering a thin layer of granulated wood pulp, or other bibulous material, then a relatively heavy layer of finely granulated depolarizing mix and then another thin layer of wood pulp. Then the whole mass is compacted into a tablet. By beveling off the edges of the tablet sufficient wood pulp is forced around the sides to insure the complete coating of the tablet. If 45 desired, the wood pulp may be mixed with flour, starch or the like, to be turned into paste when water is introduced into the cell containing the tablets. Part of the electrolyte may also be mixed with the wood pulp.

50 The invention will be more clearly under-

stood from the drawings in which Fig. 1 is a top view of a tablet, and Fig. 2 is a cross section of a part of the dry cell exemplifying various features of the present invention.

55 The tablets are indicated at 1 and each tablet is compacted of depolarizing material 2 around which is compacted an adhering coating of bibulous material 3, in the manner hereinbefore described. The tablets are provided within a zinc electrode 4 and are separated from each other by means of zinc washers 5 contacting with the zinc electrode and separated from the depolarizing material by means of the coating of bibulous material 3. A carbon electrode 6 projects through the apertures provided in the washers, the openings in the zinc washers being large enough to permit free passage 60 of the carbon electrode without contact 70 therewith.

65 It will be obvious to those skilled in the art that other methods may also be adopted for coating the tablets 1, e. g., they may be dipped in or sprayed with paste or a mixture composed of paste, granulated wood pulp and a part of the electrolyte, as described in my copending application Serial No. 688,057, filed Jan. 23, 1924.

75 What I claim is:

1. A dry cell composed of a plurality of tablets compacted of depolarizing and bibulous materials, the latter forming an adhering coating on the former.

2. A dry cell composed of a plurality of tablets each compacted of alternate layers of depolarizing and bibulous material.

3. A dry cell composed of a plurality of compacted tablets each having a covering of bibulous material on a depolarizing core.

4. In a dry cell, a plurality of tablets compacted of depolarizing and bibulous materials, the latter forming an adhering coating on the former, an electrode separating adjacent tablets, and a second electrode interconnecting said tablets.

5. In a dry cell, a plurality of tablets compacted of depolarizing and bibulous materials, the latter forming an adhering coating on the former, a zinc electrode sepa-

55

60

65

70

75

80

85

90

95

100

rating adjacent tablets, and a carbon electrode projecting through said tablets.

6. In a dry cell, a zinc container electrode enclosing a plurality of tablets compacted of depolarizing and bibulous materials, the latter forming an adhering coating around the former, zinc washers contacting with

said electrode and separating adjacent tablets, and a carbon electrode projecting through said tablets.

In testimony whereof, I have signed my name to this specification, this 22nd day of January, 1924.

WILLIAM F. HENDRY.